

L. M. Crane.

Bank-Note Paper.

No 61321.

Patented Jan 22, 1867.



Fig. 2.



Inventor.

L. M. Crane  
per *Brace & Co*  
Attorneys.

Witnesses.

Alex F. Roberts.  
Chas A. Pettit.

# United States Patent Office.

L. M. CRANE, OF BALLSTON, NEW YORK.

*Letters Patent No. 61,321, dated January 22, 1867.*

## IMPROVEMENT IN SAFETY-PAPER.

The Schedule referred to in these Letters Patent and making part of the same.

TO ALL WHOM IT MAY CONCERN:

Be it known that I, L. M. CRANE, of Ballston, in the county of Saratoga, and State of New York, have invented a new and improved Safety Record Paper; and I do hereby declare that the following is a full, clear, and exact description thereof, which will enable those skilled in the art to make and use the same, reference being had to the accompanying drawings, forming part of this specification, in which—

Figure 1 is a side view of a cylinder paper-making machine, showing the way in which my improved paper is manufactured.

Figure 2, a view of a piece of my improved paper.

Figure 3, an enlarged or magnified transverse section of the same.

Similar letters of reference indicate corresponding parts.

This invention relates to a new and improved safety record paper for wills, deeds, currency bonds, and other instruments or documents which are liable to be forged or fraudulently altered.

The invention consists in inserting in the paper pulp and incorporating with it, during the process of manufacturing the paper, one or more threads or strips of gutta percha or other material which will soften under the heat of the drying-cylinder of the paper-making machine and become inseparably united with the paper so as to be incapable of being removed or detached without destroying the latter.

In order that my invention may be fully understood I will proceed to describe the manner of manufacture.

A represents a pulp vat, and B B two cylinders, having their peripheries formed of wire cloth. C is an endless apron, constructed of felt, working over suitable rollers, D, and in contact with the peripheries of the cylinders B B. E represents two pressure-rollers, and F a series of heated cylinders. The above parts comprise an ordinary cylinder paper-making machine. The peripheries of the cylinders B B, as they rotate, take up a quantity of pulp, which is taken off by the endless felt apron C and conveyed to the pressure-rollers E, which express the superfluous moisture from the pulp, the latter being taken from the felt apron beyond the rollers E and passed around the heated cylinders F, which dry it. G represents a spool, on which a gutta-percha thread, H, is wound. This thread H passes between the two layers of felt taken by the felt apron C off from the peripheries of the two cylinders B B, (see fig. 1,) and the thread, in passing over or around the heated cylinders F, becomes heated or warmed so as to soften and unite with the fibre of the pulp and be inseparably connected or incorporated with it, (see fig. 3.) I do not confine myself to a single thread, for more may be used if necessary or desired, nor do I confine myself to a straight thread or threads, for they may be inserted in serpentine form and arranged or disposed so that the denomination of a bank note or the name of an instrument or document may be indicated by the form, shape, number, or disposition of the thread or threads. The gutta-percha thread or threads may also be made of different colors, if desired, or may be covered with colored pulp, as may be most effective to prevent counterfeiting by photography.

I am aware that paper has been manufactured with threads inserted in its fibre, but the threads have not been made of a material which will soften and unite with the fibre under the heat and pressure of the cylinders used in drying the paper or pulp.

I claim, therefore, as new, and desire to secure by Letters Patent—

The inserting or incorporating of one or more threads or strips of gutta percha, or a material possessing like properties, into the pulp or fibre of paper, during the manufacture of the same, and in such a manner that said threads or strips will be softened and firmly united to the fibre under the heat of the drying-cylinders, substantially as set forth.

I also claim, as an improved article of manufacture, a safety record paper, made substantially as herein shown and described.

The above specification of my invention signed by me this 18th day of October, 1866.

L. M. CRANE.

Witnesses:

WM. F. McNAMARA,  
ALEX. F. ROBERTS.